

## UNITED STATES PATENT OFFICE

FREDERICK G. MOSES, OF NEW YORK, RAYMOND W. HESS, OF BUFFALO, AND ROBERT L. PERKINS, OF EAST AURORA, NEW YORK, ASSIGNEES TO THE BARRETT COMPANY, OF NEW YORK, N. Y., A CORPORATION OF NEW JERSEY

## SEPARATION OF MINERALS BY FLOTATION

No Drawing.

Application filed May 20, 1927. Serial No. 193,060.

This invention relates to the separation of minerals and the concentration of ores by flotation processes, and is particularly directed to such separation and concentration carried out with the utilization of certain organic compounds containing sulfur as flotation or mineral collecting agents.

According to the present invention, improved results can be obtained in the separation of minerals and the concentration of ores by carrying out the flotation operation with the addition to the ore or mineral pulp of a thioacyl body or compound corresponding with the following formula:



where R denotes an alkyl group and X signifies a hydroxyl group or an amino group which may contain substituents. The thioacyl compounds of particular interest are those which correspond with the following formula



where R denotes an alkyl group and R' signifies a hydrogen atom or a hydrocarbon radical and more especially an aryl radical of the benzene series. Among the thioacyl compounds which may be mentioned as giving improved results in the process of the present invention are included the following: thioacetic acid,  $CH_3.CS.OH$ , thioacetamide,  $CH_3.CS.NH_2$ , thioacetanilide,



etc. The flotation agents of the present invention may be prepared by methods described in the chemical literature.

In carrying out the flotation process, the flotation agent comprising one or more of the above mentioned thioacyl compounds may be incorporated with the ore or mineral pulp in any suitable manner or at any suitable time which will insure a satisfactory flotation operation. For example, it may be introduced in the free state or as a salt into the mill in which the ore is being ground, or it may be dissolved, suspended, or dispersed in any suitable solvent or dispersing agent as, for example, in one or more of the usual flotation oils or oil mixtures, or in any suitable organic

solvent or medium, or in water or in alkali or an alkaline reagent, and the resulting solution, suspension, or dispersion incorporated with the ore or mineral pulp. While the agents of the present invention show marked action as flotation or collecting agents in ore concentration, they ordinarily possess insufficient frothing qualities and are, therefore, generally used to advantage in conjunction with any suitable or well-known frothing agent, e. g., pine oil, crude turpentine, coal tar acids, etc. They may be sometimes used to advantage in conjunction with other flotation agents. They may be used in the pure or purified state; and, in general, they may also be employed in the crude or impure state.

The process of the present invention can be carried out in any suitable apparatus, for example, those of the pneumatic type such as the Callow cell, or those where the air is incorporated with the mixture by agitation such as the Janney apparatus or the like.

It is of advantage in some cases, as with certain copper ores, to subject the ore pulp to the action of an amount of alkali sufficient to give it an alkaline reaction before subjecting it to flotation with the flotation agents of the present invention. The alkali may be caustic alkali such as caustic soda, or an alkaline salt such as soda ash, or it may be calcium oxide or hydrate. In the differential separation of various minerals, such as zinc blende from associated minerals, the presence of an alkali metal cyanide, or of copper sulfate or other salts is sometimes advantageous.

The amount of flotation agent required to be used in the flotation process will vary, it depending partly on the character and composition of the ore, partly on the particular thioacyl compound employed, and partly on other factors. Ordinarily, one-sixth to one-half pound of the flotation agent per ton of dry ore will be sufficient, but larger or smaller amounts than this may be used.

The invention will be further illustrated by the following specific examples, but it will be understood that the invention is not limited thereto. The parts are by weight.

*Example 1.*—500 parts of a copper sulfide ore (of the Miami Copper Company) assay 100

ing 1.25 percent copper was ground in a ball mill with 300 parts of water and 0.75 parts of hydrated lime (equivalent to 3 pounds per ton of ore) until practically all of it was sufficiently fine to pass through a 40 mesh screen. The ground pulp was diluted with sufficient water to give a pulp containing about 16 percent solids and subjected to flotation in a Janney mechanical apparatus with the addition of 0.0625 parts of thioacetic acid (equivalent to one-fourth pound per ton of ore) previously dissolved in an equivalent amount of normal caustic soda solution. The mixture was agitated for 30 minutes during which time about 0.06 parts of pine oil were introduced. 25.3 parts of a concentrate assaying 18.37 percent copper was obtained which is a recovery in the concentrate of 73.5 percent of the copper. The tailings assayed 0.35 percent copper. It will be noted that the equivalent of about 19.9 tons of ore was required to give one ton of concentrate.

*Example 2.*—500 parts of copper sulfide ore (of the Miami Copper Company) assaying 1.20 percent copper was ground in a ball mill with 310 parts of water and 0.75 parts of hydrated lime (equivalent to 3 pounds per ton of ore) until practically all of it was sufficiently fine to pass through a 40 mesh screen. The ground pulp was diluted with sufficient water to give a pulp containing about 16 percent solids and subjected to flotation in a Janney mechanical apparatus with the addition of 0.0625 parts of thioacetanilide (equivalent to one-fourth pound per ton of ore) previously dissolved in an equivalent amount of normal caustic soda solution. The mixture was agitated for 30 minutes during which time about 0.08 parts of pine oil were introduced. 23.0 parts of concentrate assaying 20.0 percent copper was obtained which is a recovery in the concentrate of 77.5 percent of the copper. The tailings assayed 0.28 percent copper. It will be noted that the equivalent of about 21.6 tons of ore was required to give one ton of concentrate.

*Example 3.*—500 parts of a copper sulfide ore (of the Miami Copper Company) assaying 1.21 percent copper was ground in a ball mill with 290 parts of water and 0.75 parts of hydrated lime (equivalent to 3 pounds per ton of ore) until practically all of it was sufficiently fine to pass through a 40 mesh screen. The ground pulp was diluted with sufficient water to give a pulp containing about 16 percent solids and subjected to flotation in a Janney mechanical apparatus with the addition of 0.0625 parts of thioacetamide (equivalent to one-fourth pound per ton of ore) previously dissolved in an equivalent amount of normal caustic soda solution. The mixture was agitated for 30 minutes during which time about 0.06 parts of pine oil were introduced. 27.8 parts of concentrate assaying 16.7 percent copper was obtained which

is a recovery in the concentrate of 76.0 percent of the copper. The tailings assayed 0.31 percent copper. It will be noted that the equivalent of about 18.2 tons of ore was required to give one ton of concentrate.

It will thus be noted that the present invention contemplates the utilization as flotation agents in the separation of minerals and the concentration of ores of thioacyl compounds corresponding with the formula,



where R denotes an alkyl group and X signifies a hydroxyl group or an amino group which may contain constituents; that said flotation agents may be incorporated in or with the ore or mineral pulp at any suitable time and in any suitable manner; that they may be used in the free state or as salts or in admixture with one another or in solution, suspension or dispersion in any suitable solvent or medium; and that they may be used in conjunction with other flotation agents or with frothing agents, or with both.

The present invention is of more or less general application to the treatment of different kinds of mineral substances, both natural and artificial, by flotation.

It will be further understood that the invention is not limited to the use of the particular agents or ingredients mentioned in the examples and that other agents, particularly other flotation agents of the class specified, can be similarly used.

We claim:

1. In effecting the separation of minerals, the process which comprises incorporating with the mineral pulp a thioacyl compound corresponding with the probable formula



where R denotes an alkyl radical and X signifies a hydroxyl group or an amino group which may contain substituents, and subjecting the resulting mixture to a froth flotation operation.

2. In effecting a separation of minerals, the process which comprises incorporating with the mineral pulp a thioacyl compound corresponding with the probable formula



where R denotes an alkyl group and R' signifies a hydrogen atom or a hydrocarbon radical, and subjecting the resulting mixture to a froth flotation operation.

3. In effecting the separation of minerals, the process which comprises incorporating with the mineral pulp a thioacyl compound corresponding with the probable formula



where R denotes an alkyl group and R' signifies an aryl radical, and subjecting the

resulting mixture to a froth flotation operation.

4. In effecting the separation of minerals, the process which comprises incorporating with the mineral pulp a thioacyl compound corresponding with the probable formula



10 where R denotes an alkyl group and R' signifies a hydrocarbon radical of the benzene series, and subjecting the resulting mixture to a froth flotation operation.

5. In effecting the separation of minerals, the process which comprises incorporating with the mineral pulp a thioacyl compound corresponding with the probable formula



20 where R' denotes an aryl radical of the benzene series, and subjecting the resulting mixture to a froth flotation operation.

6. In effecting the separation of minerals, the process which comprises incorporating thioacetanilide with the mineral pulp, and subjecting the resulting mixture to a froth flotation operation.

7. In effecting the separation of minerals, the process which comprises incorporating with a mineral pulp a thioacyl compound corresponding with the probable formula



where R denotes an alkyl group, and subjecting the resulting mixture to a froth flotation operation.

8. In effecting the separation of minerals, the process which comprises incorporating thioacetamide with a mineral pulp and subjecting the resulting mixture to a froth flotation operation.

9. In effecting the separation of minerals, the process which comprises incorporating with a mineral pulp a thioacyl compound corresponding with the probable formula



45 where R denotes an alkyl group, and subjecting the resulting mixture to a froth flotation operation.

50 10. In effecting the separation of minerals, the process which comprises incorporating thioacetic acid with a mineral pulp and subjecting the resulting mixture to a froth flotation operation.

55 In testimony whereof we affix our signatures.

FREDERICK G. MOSES.  
RAYMOND W. HESS.  
ROBERT L. PERKINS.